

# United States Patent [19]

Dalai et al.

[11] 3,807,993

[45] Apr. 30, 1974

[54] NICKEL BASE ALLOY CONTAINING  
HAFNIUM

[75] Inventors: Ranes P. Dalai, Stratford; Jeremy J. Walters, Trumbull; Bruce A. Ewing, Shelton, all of Conn.

[73] Assignee: Avco Corporation, Stratford, Conn.

[22] Filed: Apr. 12, 1972

[21] Appl. No.: 243,418

## Related U.S. Application Data

[63] Continuation-in-part of Ser. No. 189,733, Oct. 15, 1971, abandoned.

[52] U.S. Cl. .... 75/171, 148/32.5

[51] Int. Cl. .... C22c 19/00

[58] Field of Search ..... 75/171, 170; 148/32, 32.5

## References Cited

### UNITED STATES PATENTS

3,677,331 7/1972 Lund et al. .... 75/171

3,677,747 7/1972 Lund et al. .... 75/171

Primary Examiner—Richard O. Dean  
Attorney, Agent, or Firm—Charles M. Hogan; Irwin P. Garfinkle

[57]

## ABSTRACT

The nickel base, cobalt containing alloys of this invention contain relatively small, but nonetheless significant, amounts of tungsten and molybdenum for solid solution strengthening, chromium for oxidation and sulfidation resistance, tantalum for solid solution and carbide strengthening, aluminum and titanium to enhance the strength by precipitation of a fine dispersed phase, gamma prime  $Ni_3(A1, Ti)$ , and hafnium for intermediate strength, ductility and improved oxidation resistance.

7 Claims, No Drawings

## NICKEL BASE ALLOY CONTAINING HAFNIUM

This application is a continuation-in-part of our U.S. Pat. application Ser. No. 189,733, filed Oct. 15, 1971, now abandoned.

This invention relates to nickel base alloys exhibiting high strength, stability, ductility and resistance to corrosion, sulfidation and oxidation at elevated temperatures and which are useful for blades, vanes and integrally cast turbine wheels.

The nickel base alloys of this invention contain relatively small, but nonetheless significant, amounts of tungsten and molybdenum for solid solution strength-

A still more preferred range of compositions is as follows (in weight percent):

|   |    |           |            |           |
|---|----|-----------|------------|-----------|
| 5 | C  | 0.10-0.22 | Hf         | 0.75-1.25 |
|   | Cr | 12.2-13.5 | Ti         | 3.9-4.2   |
|   | Co | 8.5-9.5   | Al         | 3.2-3.6   |
|   | Mo | 1.85-2.05 | Ti + Al    | 7.25-7.70 |
|   | W  | 3.65-8    | B          | 0.01-0.02 |
|   | Ta | 3.65-8    | Zr         | .08-25    |
|   |    |           | balance Ni |           |

10

Exemplary alloys in accordance with the teachings of this invention had the compositions shown in Table I which follows:

TABLE I

| Heat No. | C   | Cr    | Co    | Mo   | W    | Ta   | Hf   | Ti   | Al   | Ti+Al | B    | Zr  | Ni  |
|----------|-----|-------|-------|------|------|------|------|------|------|-------|------|-----|-----|
| I        | .15 | 12.50 | 9.35  | 1.94 | 3.99 | 3.86 | 1.10 | 3.96 | 3.57 | 7.53  | .015 | .17 | Bal |
| II       | .15 | 12.50 | 9.35  | 1.94 | 3.99 | 3.86 | 2.28 | 3.96 | 3.57 | 7.53  | .015 | .21 | Bal |
| III      | .23 | 12.80 | 8.68  | 1.97 | 4.00 | 3.77 | 0.49 | 4.32 | 3.28 | 7.60  | .016 | .13 | Bal |
| IV       | .23 | 12.38 | 8.68  | 1.97 | 4.00 | 3.77 | 1.07 | 4.32 | 3.28 | 7.60  | .016 | .16 | Bal |
| V        | .23 | 12.38 | 8.68  | 1.97 | 4.00 | 3.77 | 1.55 | 4.32 | 3.28 | 7.60  | .016 | .14 | Bal |
| VI       | .23 | 12.38 | 8.68  | 1.97 | 4.00 | 3.77 | 1.80 | 4.32 | 3.28 | 7.60  | .016 | .20 | Bal |
| VII      | .23 | 12.38 | 8.68  | 1.97 | 4.00 | 3.77 | 0.44 | 4.32 | 3.28 | 7.60  | .016 | .14 | Bal |
| VIII     | .20 | 12.31 | 9.18  | 1.94 | 3.72 | 4.05 | 1.06 | 4.08 | 3.38 | 7.46  | .014 | .15 | Bal |
| IX       | .20 | 12.31 | 9.18  | 1.94 | 3.72 | 4.05 | 2.26 | 4.08 | 3.38 | 7.46  | .014 | .22 | Bal |
| X        | .20 | 12.31 | 9.18  | 1.94 | 3.72 | 4.05 | 2.16 | 4.08 | 3.38 | 7.46  | .014 | .21 | Bal |
| XI       | .20 | 12.31 | 9.18  | 1.94 | 3.72 | 4.05 | 1.16 | 4.08 | 3.38 | 7.46  | .014 | .16 | Bal |
| XII      | .19 | 12.66 | 9.42  | 1.92 | 3.75 | 3.86 | 2.40 | 4.01 | 3.27 | 7.28  | .015 | .22 | Bal |
| XIII     | .15 | 12.50 | 8.88  | 2.04 | 3.95 | 5.0  | 1.13 | 3.96 | 3.22 | 7.18  | .013 | .10 | Bal |
| XIV      | .15 | 12.50 | 8.88  | 2.04 | 3.95 | 6.0  | 1.13 | 3.96 | 3.22 | 7.18  | .013 | .10 | Bal |
| XV       | .20 | 13.35 | 8.88  | 1.91 | 3.87 | 8.0  | 1.20 | 4.18 | 3.21 | 7.39  | .012 | .11 | Bal |
| XVI      | .20 | 13.35 | 10.88 | 1.91 | 3.87 | 6.0  | 1.20 | 4.18 | 3.21 | 7.39  | .012 | .11 | Bal |
| XVII     | .20 | 13.35 | 10.88 | 1.91 | 3.87 | 7.0  | 1.20 | 4.18 | 3.21 | 7.39  | .012 | .11 | Bal |
| XVIII    | .20 | 13.35 | 10.88 | 1.91 | 3.87 | 8.0  | 1.20 | 4.18 | 3.21 | 7.39  | .012 | .11 | Bal |
| XIX      | .15 | 12.87 | 9.49  | 2.01 | 4.01 | 4.0  | 1.05 | 4.10 | 3.23 | 7.33  | .013 | .11 | Bal |
| XX       | .15 | 12.87 | 9.49  | 2.01 | 5.01 | 7.50 | 1.05 | 4.10 | 3.23 | 7.33  | .013 | .11 | Bal |
| XXI      | .15 | 12.87 | 9.49  | 2.01 | 7.50 | 5.0  | 1.05 | 4.10 | 3.23 | 7.33  | .013 | .11 | Bal |
| XXII     | .15 | 12.87 | 9.49  | 2.01 | 10.0 | 5.0  | 1.05 | 4.10 | 3.23 | 7.33  | .013 | .11 | Bal |
| XXIII    | .16 | 12.60 | 9.40  | 2.0  | 3.97 | 3.85 | 0.50 | 4.0  | 3.55 | 7.55  | .020 | .10 | Bal |
| XXIV     | .21 | 12.80 | 9.40  | 2.19 | 4.0  | 4.08 | 1.95 | 4.05 | 3.25 | 7.30  | .014 | .10 | Bal |
| XXV      | .21 | 12.80 | 9.40  | 2.19 | 4.0  | 4.08 | 1.95 | 4.05 | 3.25 | 7.30  | .014 | .15 | Bal |
| XXVI     | .21 | 12.80 | 9.40  | 2.19 | 4.0  | 4.08 | 1.95 | 4.05 | 3.25 | 7.30  | .014 | .20 | Bal |
| XXVII    | .09 | 12.30 | 9.10  | 1.87 | 7.40 | 4.94 | 1.25 | 4.18 | 3.35 | 7.53  | .012 | .12 | Bal |
| XXVIII   | .09 | 12.30 | 9.10  | 1.87 | 4.90 | 4.94 | 1.25 | 4.18 | 3.35 | 7.53  | .012 | .12 | Bal |
| XXIX     | .27 | 12.40 | 9.00  | 1.87 | 7.40 | 4.90 | 1.15 | 4.06 | 3.20 | 7.26  | .013 | .11 | Bal |

ening; chromium for oxidation and sulfidation resistance; tantalum for solid solution and carbide strengthening; aluminum and titanium to enhance the strength by precipitation of a fine dispersed phase, gamma prime  $\text{Ni}_3(\text{Al}, \text{Ti})$ , and hafnium for intermediate strength, ductility and improved oxidation resistance.

Compositions of the following analyses are contemplated as within the scope of the present invention the compositions being expressed in weight percent, the balance being Ni except for incidental impurities:

|    |           |            |             |
|----|-----------|------------|-------------|
| C  | 0.30 max. | Hf         | 0.1-3       |
| Cr | 11-15     | Ti         | 3.5-4.5     |
| Co | 8-12      | Al         | 3-4         |
| Mo | 1-2.5     | Ti + Al    | 7-8         |
| W  | 3-10      | B          | 0.005-0.025 |
| Ta | 3.5-10    | Zr         | 0.05-0.4    |
|    |           | balance Ni |             |

A more preferred range of compositions is as follows:

|    |          |            |             |
|----|----------|------------|-------------|
| C  | .25 max. | Hf         | 0.4-3       |
| Cr | 11-13.5  | Ti         | 3.5-4.5     |
| Co | 8-11     | Al         | 3-4         |
| Mo | 1-2.5    | Ti + Al    | 7-8         |
| W  | 3-5      | B          | 0.005-0.025 |
| Ta | 3.5-8    | Zr         | 0.05-0.4    |
|    |          | Balance Ni |             |

45 After vacuum melting, the alloys noted above were vacuum cast into test bars and subjected to stress rupture testing according to ASTM Standard E139. The test bars were heat treated before testing as follows: heated to 2,050° F, held at that temperature for 2 hours then air cooled, then reheated to 1,550° F and held at 1,550° F for 4 hours, then air cooled, then reheated to 1,400° F and held at that temperature for 16 hours then air cooled:

50 After the heat treatment described above, stress rupture tests were conducted on cast test bars representative of each of the heats in the heat treated condition at 1,400° F/90Ksi, 1,400° F/100Ksi, 1,700° F/39Ksi and 1,800° F/29Ksi. The results are given in Table II, it being noted that thickwall data refers to 0.250 inch diameter solid test bar results. Thinwall data refers to tubular test bar results in which wall thickness is 0.040 inch. Thickwall or solid test bar data reflects mechanical property capability of heavy sections such as might be represented by turbine blade roots. Thin wall or tubular test bar properties reflect the mechanical property capabilities of thin walled sections such as might be represented by cored or hollow turbine blade airfoils. Thinwall data are for tests at 1,700° F/35Ksi.

TABLE II

## C103 STRESS RUPTURE TEST results

| Heat No. | THICKWALL                      |           |                                |           | THINWALL                        |           |                                |           |
|----------|--------------------------------|-----------|--------------------------------|-----------|---------------------------------|-----------|--------------------------------|-----------|
|          | 1400°F/90Ksi<br>Life<br>(Hrs.) | El<br>(%) | 1400°F/95Ksi<br>Life<br>(Hrs.) | El<br>(%) | 1400°F/100Ksi<br>Life<br>(Hrs.) | El<br>(%) | 1700°F/29Ksi<br>Life<br>(Hrs.) | El<br>(%) |
| I        | 462                            | 4         | 163                            | 3         |                                 |           | 72                             | 5         |
|          | 483                            | 5         |                                |           |                                 |           | 99                             | 5         |
| II       |                                |           | 382                            | 7         |                                 |           | 79                             | 9         |
| III      |                                |           | 225                            | 5         |                                 |           | 99                             | 10        |
|          |                                |           | 87                             | 10        |                                 |           | 106                            | 10        |
| IV       |                                |           | 211                            | 5         |                                 |           | 106                            | 10        |
|          |                                |           | 180                            | 5         |                                 |           |                                |           |
| V        |                                |           | 73                             | 3         |                                 |           |                                |           |
|          |                                |           | 119                            | 5         |                                 |           | 48                             | 8         |
| VI       |                                |           | 208                            | 4         |                                 |           | 77                             | 9         |
| VII      | 277                            | 4         |                                |           |                                 |           | 65                             | 7         |
|          | 419                            | 5         |                                |           |                                 |           | 121                            | 3         |
| VIII     | 286                            | 5.5       |                                |           |                                 |           | 50                             | 8         |
|          | 408                            | 6         |                                |           |                                 |           | 37                             | 6         |
| IX       | 530                            | 3         |                                |           |                                 |           | 45                             | 10        |
|          |                                |           |                                |           |                                 |           | 38                             | 6         |
| X        | 505.7                          | 7.5       |                                |           |                                 |           | 36                             | 7         |
|          |                                |           |                                |           |                                 |           | 71                             | 8         |
|          |                                |           |                                |           |                                 |           | 50                             | 6         |
| XI       | 273                            | 4         |                                |           |                                 |           | 56                             | 7         |
|          |                                |           |                                |           |                                 |           | 60                             | 7.5       |
| XII      |                                |           | 160                            | 8         |                                 |           | 97                             | 8.0       |
|          |                                |           | 153                            | 6         |                                 |           |                                |           |
| XIII     |                                |           |                                | 97        | 5                               | 88        | 6                              | 44        |
|          |                                |           |                                |           |                                 |           | 61                             | 5         |
| XIV      |                                |           |                                | 159       | 5                               | 129       | 9                              | 61        |
|          |                                |           |                                |           |                                 |           | 58                             | 8         |
| XV       |                                |           |                                | 70        | 4                               | 53        | 4                              | 48        |
|          |                                |           |                                | 46        | 3                               | 56        | 4                              | 49        |
|          |                                |           |                                | 49        | 3                               |           |                                | 6         |
| XVI      |                                |           |                                | 104       | 8                               | 62        | 7                              | 22        |
|          |                                |           |                                |           |                                 |           | 63                             | 8         |
| XVII     |                                |           |                                | 130       | 8                               | 93        | 7                              | 27        |
|          |                                |           |                                |           |                                 |           | 38                             | 10        |
| XVIII    |                                |           |                                |           |                                 |           | 45                             | 9         |
|          |                                |           |                                |           |                                 |           | 35                             | 9         |
| XIX      |                                |           |                                | 130       | 9                               | 72        | 9                              | 37        |
|          |                                |           |                                | 103       | 8                               |           |                                | 8         |
| XX       |                                |           |                                | 149       | 4                               |           | 50                             | 6         |
|          |                                |           |                                | 174       | 4                               |           | 28                             | 9         |
|          |                                |           |                                |           |                                 |           | 64.4                           | 6.0       |
| XXI      |                                |           |                                | 142       | 4                               |           | 43                             | 10        |
|          |                                |           |                                | 224       | 5                               |           | 79                             | 5         |
|          |                                |           |                                |           |                                 |           | 81                             | 7         |
| XXII     |                                |           |                                | 224       | 5                               |           | 45                             | 5         |
|          |                                |           |                                |           |                                 |           | 101                            | N/A       |
| XXIII    | 113                            | 4         |                                |           |                                 | 39        | 4                              |           |
|          | 116                            | 3         |                                |           |                                 | 67        | 4                              |           |
| XXIV     |                                |           |                                | 144       | 9                               | 109       | 10                             |           |
|          |                                |           |                                | 167       | 6                               | 88        | 10                             |           |
|          |                                |           |                                |           |                                 | 99        | 10                             |           |
| XXV      |                                |           |                                | 181       | 15                              | 65        | N/A                            |           |
|          |                                |           |                                |           |                                 | 71        | 8                              |           |
| XXVI     |                                |           |                                | 172       | 6                               | 79        | 10                             |           |
|          |                                |           |                                | 168       | 8                               | 83        | 8                              |           |
|          |                                |           |                                |           |                                 | 80        | 9                              |           |
| XXVII    |                                |           |                                | 163       | 5                               |           | 59                             | 8         |
|          |                                |           |                                | 157       | 7                               |           | 58                             | 5         |
| XXVIII   |                                |           |                                | 130       | 4                               | 119       | 8                              | 60        |
|          |                                |           |                                | 212       | 6                               | 75        | 9                              | 10        |
|          |                                |           |                                |           |                                 | 61        | 9                              | 111       |
|          |                                |           |                                |           |                                 |           |                                | 125       |
| XXIX     |                                |           |                                | 110       | 4                               |           | 81                             | 5         |
|          |                                |           |                                | 133       | 5                               |           | 61                             | 8         |
|          |                                |           |                                |           |                                 |           | 122                            | 4         |
|          |                                |           |                                |           |                                 |           | 184                            | 4         |
|          |                                |           |                                |           |                                 |           | 212                            | 5         |
| INCO 713 | 16                             | 6         | 5                              | 4         |                                 | 20        | 12                             |           |
| MARM 421 | 50                             | 3         | 20                             | 3         |                                 | 15        | 15                             |           |
| IN792    | 255                            | 7.5       |                                |           | 75                              | 7         | 75                             | 9         |

Corresponding values for three presently known commercial alloys are appended to Table II for comparison.

INCO 713C is reported to be an alloy with a nominal 60 composition of

| C    | Cr   | Mo  | W    | Cb  | Ti   | Al   | Zr   | B     | Ni      |
|------|------|-----|------|-----|------|------|------|-------|---------|
| 0.14 | 13.0 | 4.5 | 0.20 | 2.0 | 0.75 | 5.75 | 0.05 | 0.012 | Balance |

MAR-M-421 is reported to be an alloy with a nominal composition of

| C    | Cr   | Co  | Mo  | W   | Cb  | Ti  | Al  | Zr   | B     | Ni      |
|------|------|-----|-----|-----|-----|-----|-----|------|-------|---------|
| 0.15 | 15.8 | 9.5 | 2.0 | 3.8 | 2.0 | 1.8 | 4.3 | 0.05 | 0.015 | Balance |

INCO IN792 is reported to be the alloy described in U.S. Pat. No. 3,619,182.

Table III presents the room temperature tensile properties of the alloy of this invention, heat treated as before, after casting into test bars.

TABLE III

## C103 ROOM TEMPERATURE TENSILE TEST RESULTS

| Heat No.  | Uts. (Ksi) | 0.2% Y.S.(Ksi) | El (%) | R.A. (%) |
|-----------|------------|----------------|--------|----------|
| VIII      | 181.4      | 169.2          | 3.5    | 3.2      |
|           | 172.5      | 163.9          | 3.5    | 3.2      |
| INCO-713C | 123        | 106            | 7.9    | 11.6     |
| MAR-M-421 | 150        | 130            | 3.5    | 5        |

Comparable values for the same commercial alloys are appended to the table for comparison.

In the Tables IV and V respectively, data is presented on cyclic oxidation test results conducted at 1,750° F. and hot corrosion test conducted at 1,650° F.

TABLE IV

## COMPARATIVE C103 CYCLIC OXIDATION TEST RESULTS

| Material  | Weight Change (Mg/Cm <sup>2</sup> )<br>After 240 Hours at 1750° F. |
|-----------|--------------------------------------------------------------------|
| Heat VIII | 1.15                                                               |
| Heat IX   | 0.95                                                               |
| INCO 713C | -4.40                                                              |
| MAR-M-421 | -2.20                                                              |

TABLE V

## COMPARATIVE C103 HOT CORROSION TEST RESULTS

| Material  | Depth of Attack (Mils) After 150 Hours at 1650° F. with 6 ppm Salt |
|-----------|--------------------------------------------------------------------|
| Heat VIII | 4.2                                                                |
| INCO 713C | 26.0                                                               |
| MAR-M-421 | 15.0                                                               |

It is not intended that the invention sought to be patented be limited by the foregoing description, but merely by the scope of the appended claims.

We claim:

1. A nickel base alloy exhibiting high strength, ductility, sulfidation and oxidation resistance and stability at

6 elevated temperature and consisting essentially of the following in weight percent:

|       |             |
|-------|-------------|
| C     | .30 max     |
| Cr    | 11-15       |
| Co    | 8-12        |
| Mo    | 1-2.5       |
| W     | 3-10        |
| Ta    | 3.5-10      |
| Hf    | 0.1-3       |
| Ti    | 3.5-4.5     |
| Al    | 3.2-3.6     |
| Ti+Al | 7-8         |
| B     | 0.005-0.025 |
| Zr    | .05-.40     |
| Ni    | Balance     |

2. A nickel base alloy exhibiting high strength, ductility, sulfidation and oxidation resistance and stability at elevated temperature and consisting essentially of the following in weight percent:

|       |             |
|-------|-------------|
| C     | .25 max     |
| Cr    | 11-13.5     |
| Co    | 8-10        |
| Mo    | 1-2.5       |
| W     | 3-5         |
| Ta    | 3.5-5       |
| Hf    | 0.4-3.0     |
| Ti    | 3.5-4.5     |
| Al    | 3.2-3.6     |
| Ti+Al | 7-8         |
| B     | 0.005-0.025 |
| Zr    | .05-.40     |
| Ni    | Balance     |

3. A nickel base alloy exhibiting high strength, ductility, sulfidation and oxidation resistance and stability at elevated temperature and consisting essentially of the following in weight percent:

|       |             |
|-------|-------------|
| C     | .10-22      |
| Cr    | 12.20-13.00 |
| Co    | 8.50-9.50   |
| Mo    | 1.85-2.05   |
| W     | 3.65-4.05   |
| Ta    | 3.65-4.05   |
| Hf    | 0.50-2.50   |
| Ti    | 3.90-4.20   |
| Al    | 3.20-3.60   |
| Ti+Al | 7.25-7.70   |
| B     | .010-.020   |
| Zr    | .008-0.25   |
| Ni    | Balance     |

4. A nickel base alloy exhibiting, high strength, ductility, sulfidation and oxidation resistance and stability at elevated temperature and consisting essentially of the following in weight percent:

|       |             |
|-------|-------------|
| C     | .10-22      |
| Cr    | 12.2-13.5   |
| Co    | 8.5-9.5     |
| Mo    | 1.85-2.05   |
| W     | 3.65-8      |
| Ta    | 3.65-8      |
| Hf    | 0.75-1.25   |
| Ti    | 3.9-4.2     |
| Al    | 3.2-3.6     |
| Ti+Al | 7.25-7.70   |
| B     | 0.010-0.020 |
| Zr    | 0.08-0.25   |
| Ni    | Balance     |

5. A nickel base alloy according to claim 1 which has been heat treated to produce a desired morphology of carbides and gamma prime.

6. An article formed of the alloy of claim 1.

7. A vacuum cast article consisting of the alloy of claim 1.

\* \* \* \* \*

UNITED STATES PATENT OFFICE  
CERTIFICATE OF CORRECTION

Patent No. 3,807,993 Dated April 30, 1974

Inventor(s) Ranes P. Dalai, Jeremy J. Walters, Bruce A. Ewing

It is certified that error appears in the above-identified patent  
and that said Letters Patent are hereby corrected as shown below:

Item 19 - Dalai et al. should read --- Dalai et al. ---.

Item 75 - Ranes P. Dalai should read --- Ranes P. Dalai ---.

Table II, under THICKWALL, the heading 1700°F/29Ksi should  
read --- 1700°F/39Ksi ---.

Signed and sealed this 27th day of August 1974.

SEAL)  
ttest:

CLOY M. GIBSON, JR.  
ttesting Officer

C. MARSHALL DANN  
Commissioner of Patents